

J. A. McCASKELL,  
PROCESS OF LEACHING ORES,  
APPLICATION FILED JUNE 2, 1914.

1,137,874.

Patented May 4, 1915.



(Witnesses

Jasper A. McCaskell.

*J.W. Fowler Jr.*

By T. Walter Fowler

Attorney

# UNITED STATES PATENT OFFICE.

JASPER A. McCASKELL, OF SALT LAKE CITY, UTAH.

## PROCESS OF LEACHING ORES.

1,137,874.

Specification of Letters Patent.

Patented May 4, 1915.

Application filed June 2, 1914. Serial No. 842,426.

To all whom it may concern:

Be it known that I, JASPER A. McCASKELL, a citizen of the United States, residing at Salt Lake City, in the county of Salt Lake 5 and State of Utah, have invented certain new and useful Improvements in Processes of Leaching Ores, of which the following is a specification.

My invention relates to a process for 10 leaching gold, silver, and copper ores and then regenerating the solvent.

A leading object of my invention is to 15 produce chlorin gas electrolytically from metallic chlorids (sodium chlorid preferred), and to use the chlorin thus produced to chlorinate the metals in the ore that is being treated. An aqueous solution of these chlorids is subsequently electrolyzed in the cathode side of a diaphragmed electrolytic cell, resulting in the regeneration of 20 the original chlorid solution (sodium chlorid) and the depositing of the metals in solution on the cathode.

With the above and other objects in view 25 my invention consists of the process which I will hereinafter describe and claim.

In the accompanying drawings I have shown one type of apparatus which is adapted for the carrying out of my process and 30 wherein—

Figure 1 represents a side elevation of one type of apparatus suitable for carrying out my invention, certain of the parts being shown in section. Fig. 2 is a sectional view 35 of an electrolytic cell showing the diaphragm interposed between the anode and cathode compartments thereof.

While I have shown one type of apparatus for carrying out my process I wish it 40 understood that I do not limit the process to this particular apparatus, but claim the right to use the salient steps of the process in any arrangement or apparatus where the same may be used to produce the desired 45 results.

In the apparatus shown, A, represents an agitating tank of suitable construction in which the ore is designed to be agitated in the presence of chlorin, the ore being admitted to the tank from a suitable reservoir or bin, A', which delivers the ore to an appropriate grinding apparatus, A<sup>2</sup>, where the ore is finely crushed and the powdered ore is delivered through a suitable chute or launder, A<sup>3</sup>, into the agitating tank. Associated with the grinding apparatus is a

storage tank, B, initially containing water, which tank, after the first cycle in the operation will contain the spent liquors from the anode compartment of the electrolytic cells, 60 as I will hereinafter describe, said tank having a delivery pipe, B', leading the fluid contents of the tank for admixture with the ore being reduced in the grinding apparatus.

A suitable tank or holder, F, is adapted to 65 contain chlorin and a pipe F' from this tank leads into the bottom of a vertical column, a, located within the agitating tank, A, whereby the chlorin is introduced into the bottom 70 of the column under pressure and acts as the active agent for agitating the contents of said tank, and which contents comprise the crushed ore saturated with the water, or spent liquors from the anode compartment 75 of the electrolytic cells, as before explained. The chlorin storage tank, F, is provided with a pipe, L, which leads from the upper part of this tank into the top or upper portion 80 of the agitating tank, and a pipe, K, also connects the tank, F, with the anode compartment of the electrolytic cell, there being a suitable pump, 10, introduced into the length of this pipe for delivering the chlorin gas from said anode compartment 85 back into the storage tank, F.

The electrolytic cells, D, D', D<sup>2</sup>, are each composed of suitable material and have any desired capacity and they are each provided with an impervious partition or diaphragm, 12, which is designed to act substantially as a bi-polar electrode, said diaphragm forming at one side thereof, the cathode compartment and at the other side the anode compartment, the first-named 90 compartment being provided with a suitable cathode, 13, and the second compartment having an anode, 14, said anodes and cathodes being electrolytically connected to a generator, 15, or suitable source of electric 95 current.

In the aforesaid drawing I have shown for illustrative purposes, three electrolytic cells, with the anode compartment of one cell connected to the cathode compartment 105 of an adjacent cell by suitable valve-controlled pipes, I, which connect with the bottom of the aforesaid compartments.

H represents a storage tank for an anolyte 110 consisting of water containing a small percentage of metal chlorids and which anolyte is conducted to the tank through a pipe, G,

and from the tank it is pumped through a suitable pipe, H', to the storage tank, B, before mentioned.

The agitating tank, A, has a bottom discharge which is appropriately connected to a filter press, C, of any suitable character and which is herein shown as being set at an incline, this press containing an interior carriage, C', with filter frames, C<sup>2</sup>, and said carriage being adapted to be run in and out of the tank in a manner well known in the metallurgical art, the metal chlorid solution from this filter press being delivered through a pipe, E, to a pump, E', and thence forced into the cathode compartment of the electrolytic cells through suitable branch pipes, E<sup>2</sup>, as shown.

As before stated, each of the electrolytic cells is divided into a cathode and anode compartment by means of an impervious diaphragm, 12, which serves as a bi-polar electrode as hereinafter explained. One form of this diaphragm is shown in Fig. 2, as being composed of two sheets of asbestos board, b, b', cloth, or porous earthen-ware or similar material of a porous character, and between the adjacent surfaces of said sheets and thereby rendering the diaphragm impervious is placed a thin film of mercury, c, the thickness of which is, preferably, just sufficient to keep the asbestos boards from touching, but it will be apparent that any desired thickness of mercury film or layer may be employed that is found best adapted for the carrying out of my process. In practice, the asbestos boards or other sheets between which the film of mercury is introduced may be supported by a suitable grid or perforated frame, d. In carrying out my process I do not limit the same to the use of this particular diaphragm or bi-polar electrode. In the drawings I have shown the diaphragm or bi-polar electrode as vertically disposed, but I do not confine myself to this arrangement as it is quite apparent that the same result will be obtained if the diaphragm or bi-polar electrode is horizontal and divides the electrolytic cells into the anode and cathode compartments before mentioned.

In order to make the steps of my process sufficiently clear for those skilled in the art to work the same, I will now describe the cycle of operation in treating ore. The ore is first ground to a suitable size, say from twelve to two hundred mesh, depending upon the character of the ore treated. This ground or slimy ore is delivered to the leaching or agitating tank, A, where the ore is agitated in the presence of chlorin delivered from the tank, F, in which tank the chlorin gas is stored under pressure and is delivered into the bottom of the central column, a, in the agitating tank, as before mentioned. It will thus be seen that the

chlorin gas itself is used as the agitating medium and that in my process it has the double function of agitating and chlorinating the metal contents of the ore under treatment. If the ore contains silver, sodium chlorid is added to the water used in crushing the ore and delivered from the tank, B, when first starting the operation. After the first cycle, the tank, B, will contain the spent liquors from the anode compartment of the electrolytic cells, which are derived from the tank, H, and pumped back to the tank, B, as shown. After the ore is thoroughly chlorinated in the tank, A, it is run into the filter press and the clear water filtrate obtained from the filter medium with which the press is supplied, is pumped through the pipe, E, to the cathode compartment of the electrolytic cells, D, D', D<sup>2</sup>. This filtrate contains the chlorid of gold, silver, copper, &c., in solution. The solution of sodium chlorid and the extracted metallic chlorids is admitted into the cathode compartment where the electric current dissociates the metallic chlorids into the metals which collect at the cathode, 13, and chlorin which tends to collect at one side of the mercury diaphragm, 12, the mercury diaphragm, of course, behaving as a bi-polar electrode. The sodium chlorid will also be somewhat dissociated in the cathode compartment, the sodium being deposited at the cathode, 13, where it will unite with water to form sodium hydrate and hydrogen; the chlorin will tend to collect adjacent to one side of the mercury diaphragm. The solution in the anode compartment will contain but little metallic chlorids in solution but considerable sodium chlorid which will be dissociated into chlorin which will collect at the anode, 14, and finally be delivered through the pipe, K, to the chlorin tank, F, and sodium will collect at one side of the mercury diaphragm where it will amalgamate with the mercury in the diaphragm. The sodium in the amalgam will then come into contact with the chlorin which has been liberated into the cathode compartment and form sodium chlorid, thus regenerating the original solvent agent.

From the foregoing it will be understood that my process is thus made continuous by the regeneration of the original saturated sodium chlorid solution that I started with as an anolyte. Theoretically, there should be no loss of chlorin during the cycle, but there always is a certain mechanical loss that is to be made up by adding more salt to the solution, or in other words standardizing the catholyte solution before it is sent on another cycle of operation.

In large installations, the sheets, b, b', of asbestos or like material between which the film of mercury, c, is contained, are rigidly held in place between the perforated grids,

boards or frames, but I do not confine myself to the exclusive use of asbestos, as I have used certain kinds of heavy canvas with success, and doubtless other material of 5 a more or less porous character may be used as a substitute for the asbestos. The amount of mercury used is very small as the asbestos boards, or their equivalent are placed in close relation, just so they do not touch is 10 all that is required. In practice, I have used a mercury film of about one-eighth of an inch in thickness, this being sufficient to prevent mixing of the anolyte and catholyte.

From the foregoing it will be understood 15 that my invention is a novel process for the extraction of metals from their ores and that the diaphragm which is interposed between the anode and cathode compartments of the electrolytic cells is important in the working 20 out of the complete process, and that as a result of my process I produce chlorin gas electrolytically from metallic chlorids and use the chlorin thus produced to chlorinate the metals in the ore that is being treated. 25 The anode and cathode which I employ may be of any suitable character; for instance the anode may be composed of iron, carbon, &c., and the cathode may be carbon, iron, copper, &c., as is found suitable.

30 Having thus described my invention what I claim as new and desire to secure by Letters Patent is—

1. The process herein described of leaching ores consisting, essentially, in producing 35 chlorin gas electrolytically from metallic chlorids and using the chlorin thus produced to chlorinate the metals in the ore that is being treated, and regenerating the solvent by electrolyzing an aqueous solution of the 40 chlorids in the cathode side of an electrolytic cell.

2. The process herein described of leaching ores and then regenerating the solvent, said process consisting, essentially, in producing 45 chlorin gas electrolytically from metallic sodium chlorids, using the chlorin thus produced to chlorinate the metals in the ore that is being treated, and subsequently electrolyzing an aqueous solution of the chlorids 50 in the cathode side of an electrolytic cell, thereby regenerating the original sodium chlorid, the metals in solution being deposited on the cathode of said cell.

3. The process herein described of leaching 55 ores consisting, essentially, in producing

chlorin gas electrolytically from metallic chlorids and delivering the chlorin thus produced under pressure into the body of the ore being treated for the purpose of both 60 agitating and chlorinating the metal contents of said ore, and subsequently electrolyzing an aqueous solution of the chlorids in the cathode side of an electrolytic cell and regenerating the original chlorid solution thereby.

4. The process herein described of leaching ores, which consists, essentially, in producing chlorin gas electrolytically from metallic chlorids; utilizing the chlorin thus produced to agitate and chlorinate the metals 70 in the ore that is being treated; filtering the ore and separating the liquid filtrate containing the metal in solution, and delivering said filtrate to the cathode side of an electrolytic cell; supplying the anode 75 compartment of said cell with a saturated solution of a metallic chlorid; separating the compartments of the cell by a layer of mercury; electrolyzing the cell; and storing the chlorin produced in the anode compartment of the cell and utilizing the same 80 for chlorinating the metals in a fresh charge of ore.

5. The process herein described of leaching ores which consists, essentially, in producing chlorin gas electrolytically from metallic chlorids; utilizing the chlorin thus produced to agitate and chlorinate the metals in the ore that is being treated; filtering the ore and separating the liquid filtrate containing the metals in solution and delivering 85 said filtrate to the cathode side of an electrolytic cell; supplying the anode compartment of said cell with a saturated solution of a metallic chlorid; separating the compartments of the cell by a layer of mercury; electrolyzing the cell; and delivering the sodium derived from the splitting up of the chlorid in the cell, through the body of mercury so that it acts as a soluble anode which 90 combines with the chlorin that is liberated at the cathode; and utilizing the resulting anolyte containing a small percentage of metal chlorids, for saturating a fresh charge of ore.

In testimony whereof I affix my signature 105 in presence of two witnesses.

JASPER A. McCASKELL.

Witnesses:

HARRY L. ROBERTS,  
G. F. SUMMERS.